

1

3,600,327

LUBRICATING OIL COMPOSITIONS HAVING  
IMPROVED SLUDGE DISPERSANCY  
Shih-En Hu, Westerfield, N.J., assignor to Esso Research  
and Engineering Company  
No Drawing. Filed Feb. 26, 1969, Ser. No. 802,639  
Int. Cl. C10m 1/38  
U.S. Cl. 252—32.7

7 Claims

## ABSTRACT OF THE DISCLOSURE

Mineral lubricating oil compositions are prepared containing oil-soluble additives having improved sludge inhibition and dispersion, antiwear activity, and antioxidant properties under high temperature conditions. The novel additives are prepared by reacting, at between about 215° and about 255° C., elemental sulfur with oil-soluble hydrocarbons containing aliphatic radicals and reacting the sulfurized product with primary, secondary, or tertiary mono, di or poly aliphatic amines or amino alcohols. Sludge dispersing amounts of these additives are employed in the oil compositions and usually range between about 0.05 and about 10.0 wt. percent of the total composition. They are particularly useful in lubricating oil which also contains an antiwear agent, i.e., the zinc salt of a dialkyl dithiophosphate.

## DESCRIPTION OF THE INVENTION

The present invention relates to the use in mineral lubricating oil compositions of reaction products of sulfurized oil-soluble hydrocarbons containing aliphatic radicals, either saturated or olefinically unsaturated, reacted with primary, secondary, or tertiary, mono, di or poly aliphatic amines or amino alcohols, in order to impart into the mineral lubricating oil compositions improved sludge inhibition, improved sludge dispersancy qualities, antiwear and antioxidant properties. Particularly, it is desired that such lubricating oil compositions have these qualities and characteristics where the oil compositions are subjected to unusually high temperature conditions during usage.

Numerous addition agents have heretofore been prepared for use in mineral lubricating oils including those designated as heavy duty oils which are employed in railroad diesel engines and gas engines. Prior researchers have been successful in finding various types of oil-soluble organic compounds which in one or more respects exhibit specialized and specific beneficial properties when they are incorporated into mineral lubricating oils. Thus, for many years organic compounds have been conventionally employed, in minor amounts, in lubricating oils for the purpose of lowering their pour point, improving their viscosity index, affording increased resistance to oxidation, imparting antiwear properties, inhibiting sludge formation, and dispersing sludge when it is formed during use of the oils. See British Pat. No. 1,117,500 and U.S. Pat. No. 3,018,251. Such additives have found widespread commercial use and acceptance in the oils which are conventionally employed at the present time in automotive and heavy duty internal combustion engines. A high degree of oxidative stability and an ability to efficiently disperse sludge which is formed have become essential requirements for modern-day engine lubricants. The corrosion properties, i.e., the attack of the oils and the additives contained therein on the alloyed bearings employed in today's internal combustion engines are also a factor of great significance. In particular, copper-lead and silver alloy bearings are unusually susceptible to excessive wear and corrosion difficulties. Care must be taken in the selection of additives imparting one or more

2

of the aforementioned desired properties to lubricating oils so that such compounded oils do not adversely affect the alloyed bearings employed in modern internal combustion engines.

5 A number of prior patents and pending applications recognize the beneficial effects achieved for automotive lubricating oils through the use of one or more compounds containing sulfur in chemical combination. In particular, antiwear additives are known and are commercially used which contain chemically combined sulfur.

British Pat. 1,117,500 discloses the sulfurization of polyisobutylene as well as various other polymerized alpha-monoolefins such as polyethylene, polypropylene or polybutene-1, followed by the reaction of the so treated polymer with a polyalkylene polyamine or alkylene polyamine to produce oil-soluble additives which find use as ashless detergents and dispersants in lubricating oils. In preparing the sulfurized olefin polymer wherein elemental sulfur is reacted with the polymer, temperatures of 200° C. were used in sulfurizing polyisobutylene according to the Landis article (Chem. Rev., vol. 65, pp. 237-245 (1965)) as mentioned in the left hand column of page 2 of the British patent, and a temperature of 210° C. was used for the same reaction in Example A (line 71) of the same patent. The products obtained by reacting these sulfurized polymers with the amino compounds do possess some sludge dispersant properties.

It has now been discovered that the use of oil-soluble hydrocarbons or organic compounds, particularly olefinic polymers, reacted with sulfur under specific temperature conditions and which are further reacted with a primary, secondary, or tertiary amine or amino alcohol gives rise to oil-soluble additives which when incorporated into mineral lubricating oil compositions impart to such oil compositions, unusually high oxidative stability at high temperatures, a high degree of resistance to sludge formation, a highly acceptable dispersion of any sludge that is formed during use of such oils and improved antiwear properties. What this amounts to is that the versatility of lubricating oils as to their scope of use and as to their length of use where such oils contain these novel types of additives is markedly increased so much so that even when using such compounded oils at lower temperatures or at the conventionally encountered engine temperatures, the life of the oil is increased over and beyond that heretofore attainable. Such novel compounded oils may be employed for longer periods of time, thus necessitating fewer oil changes and longer engine operation between oil changes. A heavy diesel engine operating under severe operating conditions usually requires an oil change after about 1500 hours of operation because of oxidative breakdown of the oil and excessive sludge buildup due to the high temperature conditions under which the oil is used. It is now possible to increase the life of that same oil under the same conditions by as much as 50% through the use of small amounts, i.e., 0.05 to 10.0 wt. percent, of oil-soluble organic compounds obtained from hydrocarbons, particularly polymers, predominantly of aliphatic nature, which have been sulfurized in a particular manner and which are then reacted with an aliphatic primary, secondary, or tertiary amine or amino alcohol.

The materials which may be treated with elemental sulfur or with sodium polysulfide, which is the chemical equivalent of elemental sulfur, are many and varied in number and constitute practically any and all of those oil-soluble organic compounds, some of which are polymeric or copolymeric hydrocarbons or organic copolymers of hydrocarbons with monomers containing nitrogen. Some, but not all, of these starting compounds have been added, in the past, to lubricating oils for the purpose of lowering the pour point of these oils; some, but not all,

have been added for the purpose of improving the viscosity index of the oils; and a considerable number, but not all, of these conventional polymeric organic compounds, particularly in more recent years, have been found to possess pour point depressant and viscosity index improving activities when incorporated into lubricating oils. It has now been discovered that the introduction into such organic additive compounds of elemental sulfur followed by reaction with amino nitrogen containing compounds, enhances the properties of lubricating oils when they are added thereto.

Among the many varied types of oil-soluble compounds containing aliphatic radicals which are the starting compounds and which are to be treated with elemental sulfur or its chemical equivalent are the following polymers, copolymers and hydrocarbons:

- (1) homopolymers of  $C_3$  to  $C_{18}$  alpha monoolefins;
- (2) copolymers of  $C_2$  to  $C_{18}$  alpha monoolefins with a different  $C_3$  to  $C_{18}$  alpha monoolefin;
- (3) copolymers of at least one  $C_3$  to  $C_{18}$  alpha monoolefin with a vinyl compound selected from the group consisting of N-vinyl pyrrolidone and N-vinyl pyridine; and
- (4) wax alkylated naphthalene, and wax alkylated phenol.

Exemplary of the reactants that may be employed as starting materials are the following: (copolymers are shown thus: monomer-monomer) polypropylene, polyisobutylene, ethylene-propylene, the terpolymer of ethylene-propylene-methylene norbornene, n-octene-1-isobutylene, propylene-pentene-2, isobutylene-styrene, polybutadiene, wax alkylated phenol, wax alkylated naphthalene, ethylene-butadiene, butadiene-styrene, and isobutylene-butadiene, ethylene-vinyl pyrrolidone, paraffin wax and the like.

The reaction conditions under which the oil-soluble hydrocarbons containing aliphatic radicals or the oil-soluble polymers or copolymers are subjected to reaction with elemental sulfur or with sodium polysulfide require the maintenance of temperatures between about 215° and about 255° C., preferably between about 220° and about 250° C. for a time ranging between about 30 minutes and about 40 hours, preferably for between about 5 and about 12 hours with the lower temperatures being used with the longer reaction times. The relative amounts of sulfur reacted with the oil-soluble reactants may vary considerably but are generally between about 0.1 and about 3.0 mols of sulfur, preferably between about 0.5 and about 1.5 mols of sulfur per mol of oil-soluble hydrocarbon reactant. This will result, depending upon the molecular weight of the starting material, in a final product containing chemically combined sulfur of between about 1.0 and about 10.0 wt. percent sulfur, preferably between about 1.5 and 7.5 wt. percent sulfur. Ordinarily, it is desired to employ, as a reactant, oil-soluble polymers or copolymers of at least about 400 molecular weight with the upper range being generally below 150,000 molecular weight. The preferred molecular weight range is between about 800 and about 500. The sulfurization temperature is important. A temperature below 215° C. does not produce a product which upon reaction with amine gives the improved results and a temperature above 255° C. results in excessive decomposition of the sulfurized reactant.

The product may also be prepared using a mineral lubricating oil as a reaction medium solvent or base in which the sulfurization reaction is carried out, in which case the final product constitutes a concentrate of the sulfurized reactant of between about 50 and about 80% concentration of the sulfurized compound in the base oil. This is especially useful where the reactant to be sulfurized is normally solid but oil-soluble.

The sulfurized compounds heretofore described are further reacted with organic primary, secondary, or tertiary mono, di, tri or poly aliphatic amines or amino

alcohols which may be aliphatic, or cycloaliphatic, in nature. The reaction takes place between the sulfur containing compound and the amine employed. The amino alcohols or the amines may consist of polyalkylene polyamines or their hydroxy derivatives or they may be mono, di, or triamines and the corresponding hydroxy-containing derivatives. It is preferred to employ the poly-alkylene polyamines from the standpoint of the finely achieved sludge dispersancy and inhibiting characteristics to be imparted into the lubricating oils since these types of final products have been found to be most effective for the purpose.

The polyalkylene polyamines are disclosed in some detail in the "Encyclopedia of Chemical Technology," Kirk and Othmer, volume 7, pages 22-24 (1965) second edition. In general, such amines may be represented by the formula:



wherein both  $\text{R}_1$  and  $\text{R}_2$  may be hydrogen or either  $\text{R}_1$  or  $\text{R}_2$  may be alkyl, alkylo, aminoalkyl, carbamyl, thiocarbamyl, cycloalkyl, hydroxycycloalkyl or amino.

Representative examples of the specific amino compounds which may be employed are as follows: ethylene diamine, propylene diamine, triethylene tetramine, diethylene triamine, decamethylene diamine, heptamethylene diamine, hexamethylene diamine, tetraethylene pentamine, tripropylene tetramine, pentaethylene hexamine, di(trimethylene) triamine, tetra(aminoethyl) methane, tetramethylene diamine, N-N'-dimethyl ethylene diamine, N-N'-dipropyl ethylene diamine, N-N'-diethylol ethylene diamine, N-N'-dipropylol ethylene diamine, N-N'-dimethyl butylene diamine, pentamethylene hexamine, N-N'-dimethyl amine butylamine, N-methyl-N'-propyl amylene diamine.

Additionally, amino alcohols are also useful among which the following specific amino alcohols may be employed: 2-amino ethanol, 3 - amino propanol-1, 2-amino propanol-1, di(aminoethyl) diethylol methane, 2-amino trimethylene glycol, N-ethyl - 2 - amino trimethylene glycol, 3-amino propylene glycol-1-2, 4-amino-n-butanol-1, 4-amino-n-butanol-2, N(2-ethylol)ethylene diamine, N-propyl diethylene triamine, N-N'-diethylol tetraethylene-pentamine, ethylene dinitrilo tetraethanol.

The aromatic amino compounds that are useful are of the benzene ring type and contain aminoalkyl groups attached to the benzene ring. For the purposes of the present invention, they are considered to be aliphatic amines because the amino group, or groups, are attached to an aliphatic radical. Typical compounds useful in this respect are: 3-phenyl propylamine, aminononyl phenol, aminododecyl benzene, aminoisooctyl benzene, etc.

In preparing the final amine condensation product of the sulfurized compounds, in general between about 10.0 and about 1.0 mols of sulfur, added as the sulfurized compound, are reacted with at least one amino group of the amino compound. In the case of the use of a polyamine, the same number of mols of the sulfurized compound may be employed but enough sulfur is used so that one or more amino groups present in the polyamine may be reacted.

In the amine reaction, the reaction may be carried out in a suitable solvent such as toluene, heptane and other common inert solvents, and more conveniently may be carried out using a light lubricating oil as the solvent since it is then possible to employ the final reaction product, without purification or separation, as a concentrate of 50-80% active ingredient to be added to the lubricating oil finally to be used in the internal combustion engine. Either or both of the reactants may be first placed in the solvent and after reaction the solvent is distilled off unless lubricating oil is the solvent in which case an oil concentrate is used as recovered.

In general, and in contrast to the sulfurization reaction, the condensation and coupling of the sulfurized compounds with the amine takes place conveniently at temperatures between about 80° and about 200° C., preferably between about 115° and about 160° C. for periods of time ranging between about 4 and about 30 hours, preferably between about 5 and about 10 hours. A specific preferred set of conditions involves the use of a temperature of about 120° C. and a time of reaction between about 4 and about 6 hours.

The lubricating oils are preferably mineral lubricating oils which may be derived from naphthenic, paraffinic, aromatic, or mixed crude oils. Generally, automatic crankcase oils will have a viscosity at 210° F. of between about 45 and about 90 SUS (Saybolt Universal Seconds) and at 100° F. a viscosity of between about 170 and about 1100 SUS. The viscosity indices of these oils will generally range between about 90 and about 120. In the case of high speed, heavy duty diesel engines and gas engines, lubricating oils having viscosities of between about 75 and about 80 SUS at 210° F. and at 100° F. of between about 900 and about 1250 SUS, with viscosity indices ranging between about 60 and about 80 are commonly used.

The amount of the sulfurized compound-amine reaction product which is ultimately added to the compounded oil compositions is sufficient to act, as a minimum, as a sludge inhibitor but it is also usually sufficient at the same time to serve as an oxidation inhibitor and a sludge dispersant. Generally the amount of material added will range between about 0.05 and about 10.0 wt. percent based on the total oil compositions, preferably between about 0.1 and about 5.0 wt. percent on the same basis.

The final compounded lubricating oil compositions may also contain other conventional additives. These conventional additives are designed to complement and supplement the desired properties in the final oil compositions which are attainable through the use of the novel sulfurized compound-amine reaction products.

Amounts similar to the amounts specified for the novel additive are likewise employed for the conventional additives such as corrosion inhibitors, (sorbitan monooleate), antioxidants, (N-phenyl alpha naphthylamine), pour point depressants (wax alkylated naphthalene), viscosity index improvers (polyisobutylene, or polymethyl methacrylate), antiwear agents (the zinc salt of di(C<sub>4</sub>-C<sub>5</sub> alkyl)dithiophosphate), detergents (the alkaline earth metal salts of alkyl substituted phenyl thioethers or sulfides), and dispersants (overbased alkaline earth metal salts of petroleum sulfonic acids or of alkaryl sulfonic acids) and the like.

In particular, the efficacy of the novel sulfurized compound-amine reaction product is maintained in those instances where it is added to lubricating oils that also conventionally contain the zinc salt of di(C<sub>4</sub>-C<sub>5</sub> alkyl)dithiophosphate as an antiwear agent. Unless the sulfurized compounds are prepared using temperatures of between about 215° and about 255° C., their subsequent reaction with the amino compounds seems to leave some free amino groups in the reacted mixtures. In such instances, the addition of these mixtures to lube oils, also containing the aforementioned type of antiwear agent, gives rise to a deleterious condition, in that the free or uncombined amino groups complex with the dithiophosphate compound and effectively remove it and its beneficial function by reason of the formation of a precipitate or haze that adversely affects both the antiwear and sludge dispersing properties of these additives. Such haze formation tendencies, using various sulfurization temperatures, are shown in the examples hereinafter set forth. Since the test oils therein contain the zinc salt of di C<sub>4</sub>-C<sub>5</sub> alkyl dithiophosphate (1.2 wt. percent), the nephelometer haze measurement is an indication of the degree of completeness or incompleteness of the reaction between the sulfurized polymer and the polyamine.

From this haze differential phenomenon, it is clear that the chemical nature of the sulfurized polyolefins or other hydrocarbons that are sulfurized, differs markedly depending on the specific temperature used in effecting the 5 sulfurization reaction. In turn, using the heretofore stated relative amounts of sulfurized compound and amine reactants, the type or kind of reaction is likewise dependent on the earlier used temperature in the sulfurization reaction. The haziness is due to the complex formation 10 between free amine and the zinc salt and its precipitation in the lubricating oil seems to increase in direct proportion to the type or kind of amine reaction. This character of reaction, in turn, is the result of not maintaining a temperature between 215° and 255° C. during the sulfurization reaction.

A number of routine tests were carried out on compounded oils containing the novel additives hereinbefore described, on a comparative basis.

One of these tests is known as the Sludge Inhibition 20 Bench Test. This involves the use of a sludge-containing used oil which was freed of solid sludge by centrifuging for one hour at 18,000 r.p.m. The supernatant oil was decanted from the insoluble sludge particles but the oil which was free of solid sludge particles did contain oil- 25 soluble sludge precursors which upon heating as applied in the test would tend to form additional oil-insoluble deposits of sludge. In a tared stainless steel centrifuge tube, 10 grams of supernatant used oil containing from 0.5 wt. percent to 5.0 wt. percent active ingredient to be 30 tested was heated to 300° F. for two hours in a constant temperature oil bath. Following the heating, the tube was cooled and then centrifuged for one hour at 18,000 r.p.m. gravity. The supernatant oil was decanted again from the tube and any residual deposits of sludge were 35 washed carefully with 99% n-pentane to remove all remaining oil. The weight of the solid sludge formed in the test, in milligrams, was determined. A blank run was also carried out in which no additive was employed in the oil. A substantial decrease in the amount of sludge deposited as compared with the amount deposited in the case of the blank run indicates that the additive had a sludge inhibiting effect.

Another test employed was the Cyclic Temperature 40 Sludge Test. In order to evaluate the sludge handling ability of the additives in lubricating oils in this test, a Ford 45 6-cylinder engine was used which employed a standard carburetor. It was operated at a standard speed of 1500 r.p.m.  $\pm$  15 r.p.m. under a constant load of 140  $\pm$  2 foot pounds of torque. In this test, the temperature of the oil 50 in the crankcase was cyclically and sequentially raised and lowered during the period of total hours of running the tests. The cold phase operation, i.e., the lower temperature was maintained for a period of 5 hours, alternated with a hot phase operation in which the high temperature 55 was maintained for two hours. The oil sump temperature in the cold phase was 150° F.  $\pm$  5° F. and in the hot phase operation was 215° F.  $\pm$  5° F. This test was used to determine the oxidation stability, the sludge inhibiting tendencies and the sludge dispersing tendencies 60 of the novel additive or additives.

In securing some of the following data a test known as the Falex Wear Test was also employed. This involves the use of a conventional Falex Wear Test machine which was operated with the test oils for 30 minutes using 500 pounds per square inch direct pressure, gauge, on a bearing having a rotating steel pin, which bearing was submerged in the test oil. At the end of this time, the steel pin used in the test was weighed in order to determine the amount of wear on the pin in milligrams of lost weight. This test was conducted for the purpose of measuring the amount of water which bearings would encounter under extremely severe conditions when operating in a bath of the test oil composition. Pin seizure or borderline pin seizure conditions are avoided, if possible, but 65 70 75

if they do occur, the test oil is deemed to have failed in antiwear qualities.

The Nephelometer Haze Test is designed to measure the amount of haze or light scattering arising by light reflection from the particles of a dispersed phase of a suspension, the light being Tyndall light. The intensity of the Tyndall (scattered) light passing through a liquid containing solid particles or dispersed particles produces on a photoelectric cell an accurately measurable intensity of light even at extremely low concentrations of dispersed phase. The amount of suspended solids or at least their concentration is thus capable of measurement by transmitting the output of the photoelectric cell or cells to a mirror galvanometer which, in turn, is focused on a galvanometer scale having an arbitrary index which may be standardized so as to measure various degrees of haze levels on a comparative basis. (See Operating Directions for the Coleman Model 9 Nephro-Colorimeter, D-202A, Reprinted 1956, Maywood, Ill.)

The following examples are illustrative of the characteristics of the invention but it is not intended that the invention be limited thereto.

#### EXAMPLE 1

About 500 grams of polyisobutylene of 920 molecular weight was heated with about 75 grams of elemental sulfur at a temperature of 250° C. for 6 hours. The product had a sulfur content of about 5.3%. About 100 grams of this product and about 100 grams of a solvent neutral mid-continent oil having a viscosity of about 150 SUS at 100° F. together with about 6 grams of tetraethylenepentamine were heated at 140° C. for 6 hours and thereafter stripped (with nitrogen) at 100° C. for 1 hour.

A used oil free of solid sludge particles but containing sludge precursors was subjected, with and without the use of the aforementioned experimental compounds, to the sludge inhibition bench test (SIB Test) previously described herein. The blank test run of the used oil gave 22.0 milligrams of sludge. The same test oil containing 0.4 wt. percent of the additive prepared in accordance with Example 1 gave 12.1 milligrams of sludge and in the case of the use of one-half of that amount, namely, 0.2 wt. percent of the same additive, gave 15.2 milligrams of sludge.

An automotive lubricating oil of about 9 parts having a viscosity of about 100 SUS at 100° F. and 1 part having a viscosity of about 450 SUS at 100° F. also contained the following ingredients in the following amounts (based on the total oil composition): 10.6 wt. percent polyisobutylene, 1.0 wt. percent overbased calcium petroleum sulfonate, 1.0 wt. percent copolymers of vinyl acetate and lorol fumarate and mixed with wax alkylated naphthalene, plus the below indicated amounts of a zinc salt. This oil composition was subjected to a comparative test previously described as the Falex Wear Test. In both instances the oil contained 0.6 wt. percent of the zinc salt of di(C<sub>4</sub>-C<sub>5</sub> alkyl) dithiophosphate. In the case of the oil containing no sludge dispersant additive, there was a failure. In the case of the same oil containing 3.8 wt. percent of the sludge dispersant additive of Example 1, the bearing weight loss was 1.7 milligrams which indicates an excellent antiwear activity for the additive product of Example 1.

#### EXAMPLE 2

1920 grams of the same polyisobutylene (molecular average molecular weight of 920) as used in Example 1 was reacted with 150 grams of elemental sulfur at a temperature of 250° C. for 6 hours. The product was stripped with nitrogen at 100° C. for 1 hour. 500 grams of this product, together with 500 grams of a solvent neutral mid-continent lubricating oil of 150 SUS at 100° F. and about 30 grams of tetraethylenepentamine were heated

at 200° C. for 5 hours and then stripped with nitrogen for 1 hour at 100° C.

A commercially available automotive crankcase lubricating oil of SAE 10W-30 grade which contained 75 wt. percent of solvent neutral mid-continent oil of 100 SUS at 100° F. and 8% of solvent neutral oil of 450 SUS at 100° F. was employed in a series of comparative tests previously described as the Cyclic Temperature Sludge Test. The base oil also contained about 10.6 wt. percent of unsulfurized polyisobutylene, about 1% of the zinc salt of di(C<sub>4</sub>-C<sub>5</sub> alkyl) dithiophosphate and less than 1% each of overbased calcium petroleum sulfonate and a pour point depressant which was the copolymer of vinyl acetate and lorol fumarate admixed with wax alkylated naphthalene. Each test oil had added to the base oil 3 wt. percent of a dispersant, to make a total of 100%, including the aforementioned components. The test oil that contained a commercially available sludge dispersant which was the amide condensation product of polyisobutylene succinic anhydride and tetraethylenepentamine, in the amount of 3.8 wt. percent, showed, in a Cyclic Temperature Sludge Test, a sludge merit rating for 63 hours of 9.2; for 84 hours of 6.8; and for 105 hours of 5.5. The test oil made from the same base oil to which was added 3.8 wt. percent of the product of Example 2, in place of the commercially available ashless sludge dispersant, showed a sludge merit rating at the end of 63 hours of 9.2; at the end of 84 hours of 8.1; and at the end of 105 hours of 6.2. Since a sludge merit rating of 10 represents a perfectly clean engine and a sludge merit rating of 0 represents the dirtiest possible engine, it is apparent that the additive of Example 2 exhibits improved sludge dispersancy over the commercially-available conventional additive.

Examples 3 through 15, whose data are set forth in the following table, illustrate the variables of temperature and its significance, both in inhibiting sludge and in avoiding complex formation and haze precipitation in the oil with the conventionally used zinc salt of di(C<sub>4</sub>-C<sub>5</sub> alkyl) dithiophosphate antiwear agent. In the following table, the polyisobutylene reactant (column A) had a number average molecular weight of about 920. The heading for columns E and F, SPIB-TEPA, is intended to designate reaction conditions in forming the condensation product of the previously prepared sulfurized polyisobutylene and tetraethylenepentamine. The SIB tests (columns G and H) are the same as that described in Example 1, except that the base oil alone gave 15.6 mg. of sludge and that 1 wt. percent and 2 wt. percent, respectively, of the additive were used instead of 0.2 and 0.4 wt. percent as in Example 1. The Nephelometer Haze Test (column J) was carried out in the manner previously described. The base oil employed consisted of 98.8 wt. percent of a solvent neutral mid-continent lubricating oil blend of 325 SUS @ 100° F. plus 1.2 wt. percent of the commercially marketed antiwear agent, i.e. the zinc salt of di(C<sub>4</sub>-C<sub>5</sub> alkyl) dithiophosphate. On the comparative scale used in these particular haze runs, a reading greater than 100 is unacceptable and a reading of about 43 or lower is considered to be visually clear. The blank oil was clear, having a reading of less than 9.

In carrying out the preparation of the condensation product of sulfurized polyisobutylene with tetraethylenepentamine in Examples 3 through 15, 100 grams of sulfurized polyisobutylene was dissolved in 100 grams of solvent neutral mid-continent oil of 150 SUS @ 100° F. The solution was then heated to reaction temperature and 6 grams of tetraethylenepentamine was added and the reaction temperature thereafter maintained for the indicated number of hours after which, at the same temperature, nitrogen was passed through the reacted mixture for an additional hour. The reacted mixture was then filtered hot, the filtrate constituting a reaction product oil concentrate. In the nephelometer test, 3.8 wt. percent of this concentrate was used.

TABLE

| Example | A<br>Grams<br>sulfur<br>per 920<br>grams<br>polyiso-<br>butylene | B<br>Reaction<br>tempera-<br>ture, ° C. | C<br>Reac-<br>tion<br>time,<br>hours | D<br>Sulfur<br>in<br>product,<br>weight<br>percent | E<br>Tempera-<br>ture, ° C.<br>SPIB-TEPA<br>reaction | F<br>Time,<br>hours | G<br>SIB test<br>mg.<br>sludge per 10<br>grams oil | H<br>1%<br>add. | J<br>2%<br>add. | Nephe-<br>lometer<br>haze |
|---------|------------------------------------------------------------------|-----------------------------------------|--------------------------------------|----------------------------------------------------|------------------------------------------------------|---------------------|----------------------------------------------------|-----------------|-----------------|---------------------------|
| 3-----  | 160                                                              | 210                                     | 6                                    | 7.49                                               | 120                                                  | 4                   | 17.8                                               | 22.6            | 130             |                           |
| 4-----  | 148                                                              | 220                                     | 6                                    | -----                                              | 120                                                  | 4                   | 7.5                                                | 5.0             | -----           |                           |
| 5-----  | 148                                                              | 230                                     | 6                                    | -----                                              | 140                                                  | 18                  | 4.8                                                | 4.4             | -----           |                           |
| 6-----  | 148                                                              | 230                                     | 6                                    | -----                                              | 140                                                  | 4                   | 6.9                                                | 5.4             | -----           |                           |
| 7-----  | 148                                                              | 230                                     | 6                                    | -----                                              | 160                                                  | 1.5                 | 7.9                                                | 4.5             | -----           |                           |
| 8-----  | 115                                                              | 220                                     | 4                                    | 5.27                                               | 120                                                  | 4                   | -----                                              | -----           | 43              |                           |
| 9-----  | 115                                                              | 220                                     | 6                                    | 4.79                                               | 120                                                  | 4                   | -----                                              | -----           | 36              |                           |
| 10----- | 115                                                              | 230                                     | 4                                    | 4.39                                               | 120                                                  | 4                   | -----                                              | -----           | 34              |                           |
| 11----- | 115                                                              | 240                                     | 4                                    | 4.58                                               | 120                                                  | 4                   | -----                                              | -----           | 29              |                           |
| 12----- | 94                                                               | 250                                     | 2                                    | 3.57                                               | 120                                                  | 4                   | -----                                              | -----           | 29              |                           |
| 13----- | 115                                                              | 250                                     | 6                                    | 4.56                                               | 120                                                  | 4                   | -----                                              | -----           | 22              |                           |
| 14----- | 115                                                              | 250                                     | 4                                    | 4.21                                               | 120                                                  | 4                   | -----                                              | -----           | 13              |                           |
| 15----- | 115                                                              | 230                                     | 6                                    | 4.98                                               | 120                                                  | 4                   | -----                                              | -----           | 9               |                           |

It is apparent from Example 3, Columns G and H, that the amount of sludge formed, using the product where the original sulfurization was carried out at 210° C., at 1% and 2% additions, was more than the amount of sludge formed using no additive: 17.8 vs. 15.6 mgs. and 22.6 vs. 15.6 mgs. Where sulfurization was carried out at 220° C. or 230° C. a marked reduction in sludge formation was evident, as shown in Examples 4 through 7.

Similar startling comparisons are evident as between Example 3 and Examples 8 through 15 with respect to the haze tests, in which the base oil used contained a conventional antiwear additive. Example 3, using a sulfurization temperature of 210° C., gave a nephelometer reading of more than 130, a wholly unsatisfactory lubricating oil, while products obtained from sulfurization at temperatures of 220° to 250° C. produced visually clear lubricating oil compositions.

The invention having now been fully described and illustrated, what is desired to be secured by Letters Patent is:

1. A mineral lubricating oil composition containing a sludge inhibiting amount of an oil-soluble sulfurized product prepared by reacting elemental sulfur, at a temperature of between about 215° and about 255° C., with a compound selected from the group consisting of: (1) homopolymers of C<sub>3</sub> to C<sub>18</sub> alpha monoolefins, and (2) copolymers of C<sub>2</sub> to C<sub>18</sub> alpha monoolefins with a different C<sub>3</sub> to C<sub>30</sub> alpha monoolefin and thereafter reacting said sulfurized compound with an amino compound selected from the group consisting of primary, secondary, and tertiary mono, di, and poly aliphatic amines.

2. A mineral lubricating oil composition as in claim 1 wherein the compound reacted with elemental sulfur is a homopolymer of a C<sub>3</sub> to C<sub>18</sub> alpha monoolefin and the amino compound is a polyalkylene polyamine.

3. A mineral lubricating oil composition as in claim 2 wherein the compound reacted with elemental sulfur is

polyisobutylene and the amino compound is tetraethylene-pentamine.

4. A mineral lubricating oil composition as in claim 3 wherein the compound reacted with elemental sulfur is polyisobutylene of between about 400 and about 150,000 number average molecular weight.

5. A mineral lubricating oil composition as in claim 1 wherein the amount of sulfurized compound-amine reaction product is between about 0.05 and about 10.0 wt. percent based on the weight of the oil composition, and the composition also contains as an antiwear additive, the zinc salt of a dialkyl dithiophosphate.

6. A mineral lubricating oil composition as in claim 3 wherein the amount of sulfurized compound-amine reaction product is between about 0.05 and about 10.0 wt. percent based on the weight of the oil composition and the composition also contains as an antiwear additive, the zinc salt of di(C<sub>4</sub>-C<sub>5</sub> alkyl) dithiophosphate.

7. A mineral lubricating oil as in claim 4 wherein the amount of sulfurized compound-amine reaction product is between about 0.05 and about 10.0 wt. percent based on the weight of the oil composition and the composition also contains as an antiwear additive, the zinc salt of di(C<sub>4</sub>-C<sub>5</sub> alkyl) dithiophosphate.

#### References Cited

#### UNITED STATES PATENTS

|           |         |                      |         |
|-----------|---------|----------------------|---------|
| 2,305,034 | 12/1942 | Rosen et al. -----   | 252—47  |
| 3,394,146 | 7/1968  | Hodgson et al. ----- | 252—47X |
| 3,459,664 | 8/1969  | Anderson -----       | 252—47  |

50 DANIEL E. WYMAN, Primary Examiner

W. H. CANNON, Assistant Examiner

U.S. Cl. X.R.

55 252—47, 47.5, 48.2, 48.6